

March 27, 1945.

P. SCHWARZKOPF

2,372,607

## METHOD OF MAKING LAYERED ARMORS

Filed Nov. 23, 1940



FIG. I.



FIG. 2.



FIG.3.



FIG. 4.



FIG. 5.



FIG. 6.



FIG. 7.



FIG. 8.



FIG. 10.

INVENTOR.  
Paul Schwarzkopf.  
BY J. V. Oliver.  
ATTORNEY.

BY

## UNITED STATES PATENT OFFICE

2,372,607

## METHOD OF MAKING LAYERED ARMORS

Paul Schwarzkopf, Yonkers, N. Y., assignor to  
American Electro Metal Corporation, Yonkers,  
N. Y., a corporation of Maryland

Application November 23, 1940, Serial No. 366,848

15 Claims. (Cl. 29—189)

This invention relates to the method of making an armor composed of two or more layers of different compositions, in particular of alternating layers of different structure and composition.

It has been suggested to combine a plurality of armor plates or sheets into a composite body, and also to differentiate those plates or sheets as to their composition. It has further been suggested to combine plates or sheets of armor steel with resilient or soft means in order to more resiliently receive the impinging projectile.

The invention is based on the cognition that there are other conditions to be considered besides toughness, hardness and possible resiliency of the armor. The surface conditions as well as the shape of the nose and periphery of the projectile also play a decisive role in the projectile's penetration into the armor.

Thus it is an object of the invention to give the armor qualities by which the shape of the nose and periphery of the projectile are changed while the projectile penetrates into the armor, so as to increase resistance against further penetration.

It is another object of the invention to compose the armor of layers or strata of different kinds or types of material one of which is substantially tough and hard, while the other is capable of chipping, cutting and/or grinding the nose and the periphery of the penetrating projectile.

It is still a further object of the invention to compose an armor of several alternate and bonded layers or strata of different kind or type, one kind or type of these layers or strata consisting of a hard and relatively tough material capable of cutting, chipping and/or grinding the penetrating nose and periphery of the impinging and penetrating projectile.

It is still another object of the invention to compose the armor of layers or strata of two different kinds or types of material one being primarily tough and hard and capable of resisting the penetration of the projectile to predetermined extent, while the other is primarily capable of deforming the shape of the impinging and penetrating projectile.

A still further object of the invention consists in an armor composed of bonded layers or strata of different types, one type consisting in a cast and thereafter thermally and/or mechanically treated material and the other type in a sintered hard and tough material capable of chipping, cutting, grinding, roughening or otherwise de-

forming the surface and shape of the penetrating projectile.

Still another object of the invention consists in manufacturing a composite armor of several alternating bonded layers or strata of basically different composition and structure, one kind of those layers or strata consisting of armor steel of any desired composition, the other of a hard and tough material capable of chipping, cutting and/or grinding the mantle of the projectile, and to bond the layers of the latter material with those of the armor steel during manufacture of the former.

It is a further object of the invention to manufacture a layered armor from plates or sheets of armor steel or other suitably tough and hard material, and a hard metal composition comprised of hard carbide, nitride and/or boride particles cemented by a tough and substantially metallic binder, the layers of hard metal being completed and simultaneously bonded with the preformed layers of armor steel or other hard and tough material.

A specific object of the invention is a layered armor composed of plates or sheets of armor steel and intermediary layers of hard metal of the type referred to, the hard metal being of substantially equal or lower specific weight than armor steel, and to manufacture the armor so as to effect a firm bond between the hard metal layers and the plates or sheets of armor steel.

These and other objects of the invention will be more clearly understood when the specification proceeds with reference to the drawing in which Fig. 1 shows a cross section through a piece of an armor according to the invention, Figs. 2 and 3 more schematically and in exaggeration the effect of the new armor upon the nose of a penetrating projectile, Fig. 4 more schematically a mode of manufacturing a composite armor in a continuous process, Fig. 5 more schematically a process of preparing a sheet or plate of armor steel for subsequent handling in a process according to the invention, Figs. 6 and 7 more schematically two steps of a process in which armor steel plates are combined with an intermediary layer of hard metal. Figs. 8 and 9 more schematically another manufacture of an armor composed of plates and an intermediary hard metal layer, and Fig. 10 more schematically a modification of the latter process applied to the manufacture of bent armors.

Referring to Fig. 1 the armor consists of a number of armor plates, sheets or strata 10, 11 and 12 spaced from each other, the spaces be-

tween them being occupied by layers or strata of cemented hard metal 13, 14 bonded with the adjacent plates. Assuming that a projectile 15 arrives in the direction of arrow 16 and rotates in the direction of arrow 19 around its axis, the projectile will first percuss plate 10 and thereafter penetrate into layer 13. While the nose of the projectile digs into layer 13, the hard particles, such as of carbides, contained in the cemented hard metal will work upon the surface of the nose and cut, chip, grind, roughen and deform it. The projectile 15 may be deformed thereby as shown in Fig. 2. The thus deformed nose of the projectile thereafter percusses armor plate 11 and penetrates into the cemented hard metal layer 14. Thereby the nose is further deformed, roughened, cut, chipped and/or ground, and assumes the shape as shown in some exaggeration in Fig. 3.

It will be appreciated that by the percussion of plate 10 the speed of the projectile is somewhat decreased and some kinetic energy stored therein consumed. By working its way through the cemented hard metal layer 13, the speed and kinetic energy of the projectile is further reduced and in addition thereto another part of its kinetic energy consumed by the deforming, cutting, chipping or grinding action of the hard metal upon the surface of the nose of the projectile.

Simultaneously the aptitude of the projectile to further penetrate into and percuss the armor is considerably reduced by that deformation of its nose and roughening of its surface.

It is well known that the mantles of projectiles are made as hard and smooth as possible, in order to facilitate penetration of an armor. Sometimes metals of relatively low melting point, such as cadmium, are used as coating or cover of the mantle; when the armor is hit, the metal is instantaneously heated to a high degree, it melts and acts like a liquid lubricant on the mantle, while the projectile penetrates into the armor. The purpose of the cemented hard metal layer or layers according to the invention is primarily to deprive the penetrating projectile of its smoothness, as well as of its shape proper for further penetration. It also serves to abrade any lubricant material from the mantle. Furthermore, any deformation, roughening or abrading action consumes part of the kinetic energy of the projectile, and all these factors combined result in the reduction of the penetrating power of the projectile to a considerably higher degree, as it would be the case of instead of a cemented hard metal layer, according to the invention, a plate or layer of armor steel of equal thickness and weight were provided.

Reverting to Fig. 1, it will now be understood that penetrating of armor plate 11 is more difficult for the projectile than of the first armor plate 10; the projectile is somewhat deformed and roughened, and its lubricant abraded.

Due to this deformation of the nose and considerable loss of kinetic energy in passing the cemented hard metal layer 13, plate 11 will be capable of more effectively resisting penetration by the projectile and to again reduce the speed or kinetic energy still stored in the projectile.

Upon penetration into the second cemented hard metal layer 14, another deforming or roughening action is exerted upon the nose of the projectile; due to its considerably reduced speed of the projectile penetrates cemented hard metal layer 14 more slowly and can be more effectively worked upon by the cemented hard metal in the

sense described above. This results in an additional and more considerable deformation of its nose, as shown somewhat in exaggeration in Fig. 3.

5 Depending upon the size and energy stored in the projectile, it will be sufficient to provide three layers of armor steel with two intermediary layers of cemented hard metal, as shown in Fig. 1, to stop the projectile in or on the armor plate 12.

10 It will be further appreciated that according to the size of and stored energy in a projectile intended to be resisted by an armor, the number of armor plates and intermediary cemented hard metal layers can be increased to the effect described above, or reduced to one cemented hard metal layer or stratum backed by one layer of steel; sandwiching of a cemented hard metal layer or stratum between two layers or strata of steel is however preferred.

15 20 As to the composition of the armor steel plates or sheets, in general any known composition can be used, such as hard and tough alloy steel e. g. chromium steel, nickel steel, manganese-nickel-steel, molybdenum-nickel-steel, manganese steel, phosphorus steel; however, low carbon steel preferably relaxed and not springy, such as steel known as "U. S. Steel COR-TEN," hot rolled and relaxed low carbon steel, and not or only slightly alloyed with other additions, is preferred. It is

25 30 common to those materials to be manufactured by casting and subsequently thermally and/or mechanically treating them, such as hardening, annealing, hot and/or cold rolling, forging, etc. There may also be used layers or backings of

35 tungsten, molybdenum or alloys thereof, preferably in the form of sheets.

40 As a cemented hard metal layer a sintered composition opposed to a molten composition is used. Molten compositions require relatively high temperatures for their manufacture, and their bonding with armor steel of known composition is impossible without melting and ruining at least the shape of the latter. As such sintered

45 hard metal compositions, those of carbides, nitrides or borides of tungsten, molybdenum, chromium, tantalum, niobium, vanadium, titanium, zirconium and boron are usable. Due to their low specific weight, extreme hardness and availability in this country, carbide, nitride or boride

50 of titanium are preferred. Any suitable mixtures of any two or more of the compounds referred to and preferably combined into compounds or solid solutions of even greater hardness can be used. As a binder for the hard particles tough materials, such as cobalt, nickel and iron are preferred, however for reasons to be set forth later on, also

55 alloys can be applied using iron as a base and cobalt, nickel, copper and aluminum as additions; there may further be used an alloy such as of copper and nickel, copper and cobalt, etc. All these binders or cementing materials have considerably lower melting temperatures than the carbides, borides or nitrides. The latter are first

60 to be prepared from the chosen metal basis in well known processes and thereafter to be comminuted to desired particle size. In contradistinction to hard metals as known and used for tool materials, the invention is not so much concerned with extremely fine and uniform particle sizes;

65 though particle sizes averaging from 5 to 30 microns may be used to advantage for light armors and thin hard metal strata, larger particle sizes, up to 100 micron and more are preferred for heavier armors or thicker hard metal layers.

70 75 It will be appreciated that with the invention

no effect comparable with normal machining of a work is attempted, the latter resulting in accurately shaping the work and smoothing and equalizing its surface. According to the invention, the smooth surface and given shape of the nose of the projectile should be removed as fast and thoroughly as possible, the nose cut, chipped, ground and torn off, and regularity and smoothness of the thus worked upon nose of the projectile would be just contrary to this purpose.

Hence destruction of smoothness and regular shape of the worked upon nose of the projectile is an object of the invention, as opposed to the desired action of any tool material. Angular shapes of hard particles, resulting from crushing and short ball milling are preferred, as opposed to as fine as possible grinding and consequently rounding off of hard particles to be used in tool materials.

While the binder in tool materials is to give 20 toughness to the tool so that it can be used for a long period of time without losing its shape, and can sustain a great many shocks during machining, with the invention conditions similar to those prevailing with tool materials do not exist. The binder serves to cementing, i. e. firmly hold the particles in their position and to connect the adjacent armor plates. When the cemented hard 25 metal comes into action, i. e. a projectile penetrates into it, this only occurs once and is to the effect of at least partly destroying the layer. Hence no views as to a long life time and sustaining a great many consecutive shocks apply to the binder.

Under the impact of the projectile, the hard 30 metal layer will crack locally, and the great mass of hard particles contained therein will act upon the projectile, whether they are still bonded together or not. If firmly held in place, they will cut into and tear the surface of the mantle; if they become loose, they will act like blasts of extremely hard sand or abrading powder upon the nose. No time is given to any locally loosened parts to fall off their backing plate or sheet, or to dodge aside.

The armor steel plates backing each hard metal layer will assist in keeping the hard metal, still bonded or locally cracked, in its place, and thus operate not only as individual obstacles to the penetration of the projectile when it reaches that plate, but in addition thereto as an effective backing of the hard metal in front of it.

This cognizance of the invention is of extreme importance for facilitating manufacture of an armor according to the invention.

It has been mentioned above that hard particle sizes of about 5 to 30 microns are advantageous for relatively light and thin armors. It is understood that relatively light armors afford protection only against relatively light projectiles having little mass which can store relatively little kinetic energy. It is obvious that a great many of the extremely small hard particles will be hit simultaneously by the nose of the projectile when it impinges the armor. The fine hard particles will not crack under the impact anymore. The metal binder cementing them cannot be softened by the relatively small amount of heat developed by the impact, and firmly holds the hard particles hit. Thus the nose of the impinging projectile will be deformed and flattened by the hard particles hit; if the nose is somewhat elastic, the projectile will be repelled like an elastic ball, and if the nose is not elastic, the projectile will be stopped

and fall to the ground. In any event such light projectiles cannot penetrate the cemented hard metal layer or detrimentally indent it, and consequently the layer and its backing can be made relatively thin and correspondingly light in weight.

As a binder any material as mentioned above can be used. Soft pure iron (ferrite) is of particular utility for reasons to be set forth later on.

- 10 In general the cementing binder is also powdered and intimately admixed with powdery hard particles to form the initial mixture from which the layer is to be made. The size of the particles of the binder should advantageously be as small as possible in order to facilitate production. Sizes from 3 to 30 microns are therefore preferred, though larger ones may be used.

As to the ratio of hard particles and binder, the specific weight or volume of the former must be considered. The smaller the specific weight, the smaller should be in general the relative amount by weight of those hard particles. While with tungsten carbide which is of a specific weight of 15.5, amounts of a binder of between 9% to 15% (or higher) are preferred, with titanium carbide which is of a specific weight of only 4.2, an amount of binder between about 15% to 30% (and higher) is preferred. These ratios are given with reference to binders selected from the iron group. Should the binder be e. g. of an alloy or metal of lower specific weight than the iron group metals, the relative amount of the binder should be accordingly reduced.

In general therefore, for hard particles and binder materials of the kind recited above, a ratio of from 91% to 60% by weight of hard particles and from 9% to 40% binder may be given, without limiting however the invention to any particular ratio or range.

- 40 Referring to Fig. 4, the manufacture of an armor, consisting of sheets of e. g. relaxed low carbon armor steel of a thickness of about 1/25" to 1/10" and intermediary layers of hard metal of the same or greater thickness shall be described by way of exemplification. From a supply roll 16 of steel sheathing, a sheet 17 is drawn off by means of rollers 18, 19, pressed against the sheet and driven in the direction of the arrows with predetermined and preferably adjustable speed. The sheet travels in the direction of arrow 22 into a unit 26 (indicated in dotted lines) comprising a hopper 20 filled with a powdery initial mixture and provided with a propeller or other means for depositing predetermined and preferably adjustable amounts of the initial powdery mixture during a unit of time, in a layer of desired thickness onto sheet 17. Roller 23 is pressed from above upon the exposed surface of layer 21 and backing roller 24 from 50 below onto the lower surface of sheet 17. Thereby the hard metal powder is spread uniformly over and pressed into the sheet. Depending upon the pressure exerted by rollers 23, 24, more or less compacting of the layer and superficial 55 mechanical uniting with sheet 17 can be obtained even in the cold. Pressures of the order of 15 tons p. s. i. generally suffice if finest powders of cobalt, nickel or ferrite form the binder.

- Rollers 23, 24 can either be heated or separate heating means can be arranged behind them. If the rollers were heated for instance by an electrical resistor (not shown), placed inside them or their shafts, some compacting of the layer and its superficial bonding with the sheet 75 can be obtained by pressure on the rollers of

an order of 2 to 5 tons p. s. i. Such compacting will also be arrived at while the layer and sheet pass furnace 25. Temperatures from 500° to 700° C. should not be exceeded in order to prevent undesirable oxidation and to avoid needless waste of heat; if higher temperatures are desired to be applied in order to effect presintering, or if for other reasons advisable, a protective atmosphere can be used in furnace 25 and along the following path of the sheet and layer thereon.

If desired, any number of units similar to unit 26 can be arranged behind it; one such unit 26 is indicated in dotted lines. In those units, arranged in series, either exactly the same conditions can prevail, or the pressure exerted by rollers 23, 24 can be raised from unit to unit, and/or the temperature of furnace 25 raised from unit to unit to the desired maximum. Such series arrangement of units is preferred if layers of greater thickness are to be applied.

Sheet 17 provided with layer 21 of desired thickness and preferably compacted, travels now under supply roll 27 of a sheet of armor steel of the same or different composition, same or different thickness as sheet 17.

A sheet 28 is wound off supply roll 27 by rollers 29, 30 driven in the direction shown by arrows and pressed from above and below against the upper side of sheet 28 and the lower side of sheet 17, respectively. The pressure should be sufficiently high (a few tons p. s. i.) in order to firmly set sheet 28 upon layer 21. The two sheets 17 and 28 with intermediary layer 21 now travel through a furnace comprising a heating chamber 30 and a cooling chamber 33. The heating chamber is formed by a preferably tubular refractory 32 in which electrical resistance heaters 31 are inserted. The latter may consist of suitable material of sufficiently high melting point such as tungsten, molybdenum, etc., as well known in the art. By adjusting the heating current any desired temperature can be obtained within chamber 30. Any other type of furnace, such as of the induction type, can be used.

The temperature in chamber 30 should be such that the initial hard metal mixture is sintered. Depending upon the nature of the binder, the sintering temperature in chamber 30 should be kept between about 1000 to 1350° C., and in any way substantially below the melting point of the armor steel sheet used, and above about 900° C.

During sintering of the binder, also diffusion or coalescing between the binder and adjacent surface layers of the sheets 17 and 28 occurs, securing a firm bond between the binder and thereby the hard metal layer 21 and those sheets.

During the travel of the combined sheets and layer now forming a unit through chamber 30 sintering is completed, and cooling starts while they travel through chamber 33. Cooling is effected by a cooling jacket 34 passed by a suitable cooling or refrigerating medium. Jacket 33 may be subdivided in order to exert a staggered cooling action according to a desired cooling curve upon the sintered unit passing it. By suitable dimensioning the length of chamber 33 with respect to the speed of travel of the unit through it, any desired heat treatment can be applied, particularly to sheets 17 and 28. It should be understood that at high sintering temperature any particular quality imparted to the steel during its manufacture may be lost, but reinstated by the heat treatment in chamber 33. Thereby fast or slow cooling, or first fast and then slow cooling, or vice versa, can easily be effected.

It should be understood that the process as illustrated in Fig. 4 can be multiplied in any desired way. The temperature in a heating chamber 30 can be kept below 1000° C., thus effecting

5 only a preliminary bond between sheet 28 and the layer 21 compacted or presintered upon sheet 17, and the unit so obtained may be pushed into another one or into a series of units 26 in which another powdery layer is deposited upon sheet 10 28 and compacted or presintered thereon. Thereafter another sheet of armor steel may be positioned upon that second upper layer in the way shown for sheet 28, and this repeated until 15 an armor of any desired number of sheets and intermediary powdery and compacted layers is composed. The thus composed entity is then passed through a furnace of the type of furnace 30, 33 in which final sintering and cooling is done to the desired effect of having all the sheets of 20 armor steel and all the compacted layers of hard metal sandwiched between and bonded with them.

It is evident however that sheets 17, 28 with intermediary finally sintered layer 21 can be introduced in another process in which another layer of hard metal and another sheet is added to it in a similar process, and these processes can be multiplied until finally an armor consisting of 25 a desired number of armor steel sheets and intermediary sintered layers of hard metal sandwiched between and bonded with them is obtained.

It is also evident that instead of heating rollers 23, 24 or rollers 29, 30, and instead of or in addition to furnaces 25 any other heating means can be used, such as rows of acetylene-oxygen burners arranged above and across the exposed surface of layer 21, as indicated in dotted lines at 30 52 and 53. The flame of those burners has to be regulated so as to effect the desired heating and may be of oxidising, deoxidising, or neutral character in order to either oxidise e. g. superfluous carbon, if present, or to remove undesired oxide films if formed on the powdery particles of 40 the layer, or not to affect them at all.

In order to prevent oxidation, or to deoxidise the exposed surfaces of sheets 17, 28, a suitable gas can be led through chambers 30 and 33. To this effect a hood 35 is provided at the entrance 50 of chamber 30 closing as near as possible to the sheets, and a suitable gas, such as hydrogen, carbon monoxide or dioxide, hydrocarbons, cracked gases, etc. is introduced through tube 54 and released at the other end 56 of the furnace where 55 they may be burned off.

Assuming that powdery pure iron (ferrite) is used as a binder, its melting temperature is about 1530° to 1550° C., and its presintering temperature is therefore about 1100° C.; it starts to become plastic at about 100° lower, so that within the unit 26 a temperature up to 900° C. or somewhat higher can be applied if presintering is desired. In chamber 30 a temperature above 1100° C., but below 1300 to 1350° C. which is the melting point of low carbon steel, should be applied. At such temperatures complete sintering of the ferritic iron can only be obtained if the ferrite powder is extremely fine and the period of sintering 60 extended to between 2 and 4 hours. However, complete sintering is not a condition of the invention. Even a still somewhat porous hard metal will suit the purpose of the invention, since the ferrite combines with the steel at considerably lower temperatures and secures a bond between the binder and the armor steel sheets firm 70 75

enough for mounting the plate on stationary or mobile objects, such as tanks or aircraft. As pointed out above, no substantial mechanical force is acting upon the hard metal layer comparable in any respect with the strain exerted upon tool materials in machining a work. At the moment of impact of the projectile however the bond afforded also by a more or less porous binder will suffice.

If nickel is used as a binder, presintering temperatures of about 1000° C. are sufficient, and nickel plastifies sufficiently and below 900° C. so as to obtain a compact of the hard metal layer. High sintering temperature of nickel is about 1300° C. and consequently temperatures from between 1200° to 1300° C. in chamber 30 will suffice for even highly and completely sintering the nickel binder and bonding it to the armor steel sheets within a period of sintering from about 45 minutes to two hours.

Similar views apply to the use of cobalt, the presintering and sintering temperatures of which are only a few degrees higher than those of nickel.

In connection with the above it should also be considered that the presintering and sintering temperature of the metals dealt with are somewhat lowered by the presence of the interspersed hard particles, thus securing the effect of the invention. However, if alloy steels of particularly low melting point are used for the armor steel plates or sheets, composite binders can be used, as mentioned above, or stellite.

The sintering temperature of ferritic iron can be reduced by about 100° by the admixture of about 20% copper, and a higher percentage of copper further reduces those temperatures. Diffusion temperatures of copper and iron can be found even below 1100° C., and thus in chamber 30 the copper admixed to the binder will diffuse into the armor steel sheets and thereby assist in creating a firm bond.

In a similar way, by admixture of 20% aluminum to pure iron, its sintering temperature can be reduced by about 100° C., and the aluminum diffuses and bonds together the iron particles as well as the iron with the armor steel at far lower temperatures, about 820° C., if 20% aluminum is admixed, and thus assists in creating a bond between the hard metal layer and the steel sheets even during presintering, the temperatures of which can be kept accordingly low.

If nickel is used as a binder, remarkable reductions in the sintering temperatures can be attained by the addition of chromium. An admixture of 35% chromium reduces the sintering temperature by at least 50° C. and an admixture of 43% chromium lowers the presintering and high sintering temperatures of nickel by more than 150° C. Higher chromium admixtures still further lower the sintering temperatures.

The admixture of chromium has the effect of hardening the binder which is highly objectionable with hard metals for tool materials, while it is desirable for the purposes of the invention.

By admixing 20% copper to nickel its sintering temperature can be lowered by about 50° C. and larger admixtures of copper further lower those temperatures. Since copper diffuses into iron below 1100° C., it is evident that a firm bond between the nickel-copper binder and the steel sheets of any description can be effected by admixing copper.

It should be understood that the above are only a few examples for illustrating the possibili-

ties and advantages of the invention and its utter difference from the uses ordinary hard metal can be put to.

In order to increase the bond between the binder and the sheet, the surface of the latter to be contacted by the hard metal layer can be roughened in any way desired, such as mechanically sand blasting, and/or any chemical or electro-chemical etching treatment. By mechanically roughening, the exposed surface can be enlarged to twice its original size and by etching to even five times its original size. In the latter case the surface becomes extremely porous and facilitates permeation of the plastified binder during sintering. In addition, the enlarged surface greatly assists diffusion. Portions of the binder penetrating the pores are quasi mechanically anchored in it and the strength of the bond is additionally increased. The irregular valleys and ridges obtained by mechanical roughening also serve to increase the surface for diffusion and mechanically bonding the plastified and pressed on binder, cementing the hard particles.

Another way of assisting the bond consists in plating the armor steel sheet with a suitable metal, such as iron, sponge iron, copper, nickel cobalt, Monel metal, alloys of copper, iron, copper cobalt, copper nickel, iron nickel, nickel vanadium, copper vanadium, etc. To this effect an arrangement as illustrated in Fig. 5 can be used.

Here again a sheet or plate 54 can be moved by means of driven feeding rollers 55, 56, below a hopper 57 filled with the desired finest powdery metal or alloy as exemplified above and driven in adjustable quantities by propeller 58 through the discharge opening of hopper 57, so that an extremely thin layer 59 is deposited and spread over sheet or plate 54. The sheet is moved through a heating chamber 60 and cooling chamber 61 of a furnace 62 provided with cooling jacket 63, the structure of which is substantially the same as of heating chamber 30 and cooling chamber 33 of Fig. 4. Again a hood 64 can be provided into which protective gas is led through tube 65 and released at 66. The temperature within the chamber 60 should be kept below about 700 to 900° C., but above about 450° to 500° C., the same way as in the compacting or presintering unit 26 of Fig. 4.

Due to the extreme fineness of the powder and thinness of the layer, plating at such low temperature can be achieved even without pressing the layer upon the sheet before or after heating, though pressure rollers like rollers 18, 19 in Fig. 4 can similarly be provided in the apparatus and used in the process illustrated in Fig. 5.

The thus or in another way well known in the art plated or coated sheet or plate is then used in any process herein described, e. g. as sheets 17, 28 or plates 38, 44, 67, 81, the plated or coated surface to be on the side where the hard metal layer or stratum is to be applied. If a sheet or plate is sandwiched between two hard metal layers the plate or sheet is to be plated or coated on both sides.

In order to manufacture an armor of stiff plates, a process as illustrated in Figs. 6 and 7 can be used. Plate 67 is positioned on supporting rollers 68 and driven by another roller 69 in the direction of arrow 70. The plate passes under a hopper 71 provided with propeller 72 and filled with the powdery initial hard metal mixture. A layer of the powdery mixture is deposited on the plate and preferably heated pressure rollers 73, 74 compact the layer on and onto the plate. The

whole is then passed through furnace chamber 14 and cooling chamber 15 the structures of which need not be explained in detail any more. Protective gas is led in through tube 16 and hood 17 and released at 18. The temperature within chamber 14 should be between 500 to about 900° C. in order to further compact or presinter or frit the hard metal layer and bond it to some extent to plate 37. Pressure may be exerted upon it while still hot, but below about 500° C., by pressure rollers 19, 20.

Upon this unit another armor steel plate 21 is positioned and the so sandwiched plates and hard metal layer positioned on supporting rollers 22 and pushed through another furnace chamber 24 and cooling chamber 25 in a protective atmosphere admitted through tube 26 and hood 27, and released at 28. In chamber 24 sintering at temperatures above 900° and 1000° to below 1350° C. is effected during a suitable period of time, the same way and to the same effect as described with reference to Fig. 4, and in cooling chamber 25 which may be subdivided for the purpose set forth above, any desired annealing or other heat treatment of the steel plates can be effected. The armor leaves the furnace in this case the same way as in the continuous process described above at a temperature below 900° C. and preferably below 500° C. It should be understood that any number of plates and hard metal layers can be combined in the way described. Any hard metal layer deposited upon a plate should be heat treated at or below about 700° to 900° C. for compacting and presintering, if desired, another plate positioned and pressed thereon, etc., and the unit consisting of the desired number of layers and plates then finally compressed and sintered.

If the sheet-like armor obtained in a process as illustrated in Fig. 4, or the plate-like armor illustrated with reference to Figs. 6 and 7, is to be cut to shape thereafter, this should be done while it is still hot, preferably immediately after it leaves the last sintering furnace.

Another way of manufacturing armors comprising stiff plates is illustrated in Figs. 8 and 9. A die 37 is used, provided with recesses 38, and armor plate 39 is positioned in the die. Thereafter a hopper 40 containing a powdery initial hard metal mixture 43 and provided with a propeller 42 for the purpose set forth above is moved to the right in the direction of the double arrow 41 over the die. While above the opening of the die, propeller 42 is rotated and a layer of hard metal deposited upon plate 39 in the die. The hopper may be moved any desired number of times back and forth over the opening of the die, until a number of powdery layers is deposited thereon giving the desired thickness of the sintered hard metal layer, considering in this case the same way as in those described above the shrinkage during sintering (or presintering). Thereupon another plate 44 is positioned in the die, pressure plate 45 is lowered in the direction of the arrow in Fig. 8, the whole is compressed (25 to 100 tons p. s. i.) and in this example heated by induction heating to sintering temperatures above 900° C. and preferably between about 1000 to below 1350° C. Coils 46 are provided for this effect. Heating and pressing may be effected simultaneously or alternatively and repeatedly. Pressure member 45 may also be used like a drop hammer.

Before plate 44 is inserted, and while the die is still open, plate 39 and layer 43 deposited there-

on may be heated to a temperature below 700° to 900° C. in order to effect compacting or presintering of the powdery initial hard metal layer, and some shrinking and degasification. The sintered armor is removed by angular instruments inserted through recesses 48.

Here again any number of plates and hard metal layers can be combined in the way described above. If a curved armor is to be produced, a die 50, Fig. 10, can be used, upon which the precured armor plate 49 is positioned. Subsequently a powdery initial hard metal layer 51 is deposited upon plate 49, principally in the same way as described with reference to Fig. 8. However, in this case some binder (about 1 to 6% by weight), such as water, dextrine, glycerine, glucose should be admixed to the powder in order to render it plastic. Instead of using a propeller in hopper 40, a piston 52 then should be used which is pressed downwardly at predetermined speed, pushes out the plastic initial hard metal powder, and desposits it upon plate 49. After the powdery initial hard metal layer of desired thickness (considering considerable shrinkage) is thus deposited, heat is applied by induction coil 46 to at least 200° C., but preferably to below 700° to 900° C. in order to drive off any volatile matter of the binder and simultaneously sufficiently compact or presinter the layer 51 on and onto plate 49, to degasify it and to effect considerable shrinking. Thereupon plate 50 is inserted in the die and processed and finally sintered in the way described with reference to Fig. 8, or any number of additional hard metal layers and plates applied and the whole then finally pressed and sintered in the way described above.

It should be understood that the invention is not limited to any preferred features described hereinbefore, but to be derived in its broadest aspects from the appended claims.

What I claim is:

1. A process of manufacturing a layered armor composed of a number, two as a minimum, of layers or strata of different type material, a first type being ferrous, tough and hard and including in its manufacture a casting step, while the second type of material consists of a sintered hard metal composition obtained by sintering an initial mixture of hard particles selected from carbides, nitrides and borides of at least one element selected from the group consisting of tungsten, molybdenum, chromium, tantalum, niobium, vanadium, titanium, zirconium and boron, and a powdery cementing metal of lower melting point than said particles, said cementing metal always including an appreciable amount of iron group metal, comprising the steps of depositing at least one layer of said initial mixture upon said first type layer, compacting said deposited layer upon a completed layer of the first type, and finally heating said layers to temperatures between about 900° to below 1350° C. until said mixture is finally sintered and essentially simultaneously firmly bonded with said first type layer.

2. In a process as claimed in claim 1, the step of heating the deposited layer on said completed first type layer to below about 900° C. before subjecting them to final sintering.

3. In a process as described in claim 1, the step of presintering said deposited layer upon said completed first type layer, before final sintering.

4. In a process as described in claim 1, heating the deposited layer to a temperature below about

700° to 900° C. and compressing it previous to final sintering.

5. In a process as described in claim 1, the step of roughening the surface of said completed first type layer to be bonded with said second type layer before applying the latter.

6. In a process as described in claim 1, the step of coating a surface of said completed first type layer to be bonded with said second type layer, with a bonding metal composition essentially consisting of an appreciable amount of chromium and a balance selected from iron group metal, before applying the said second type layer.

7. A process of manufacturing a layered armor composed of a number, two as a minimum, of layers or strata of different type material, a first type being ferrous, tough and hard and including in its manufacture a casting step, while the second type of material consists of a sintered hard metal composition obtained by sintering an initial mixture of hard particles selected from carbides, nitrides and borides of at least one element selected from the group consisting of tungsten, molybdenum, chromium, tantalum, niobium, vanadium, titanium, zirconium and boron, and a powdery cementing metal of lower melting point than said particles, said cementing metal always including an appreciable amount of iron group metal, comprising the steps of continuously feeding a completed first type layer under means for depositing thereon a layer of an initial mixture for said second type layer and depositing said second type layer on said completed first type layer, feeding said layers into means for compacting said deposited layer upon said first type layer, thereafter successively passing said layers through heating zones of different degrees of temperature, in the first of which said deposited second type layer is heated to a temperature below about 700° to 900° C. and in the last of which said deposited layer is heated to final sintering temperature and thereby finally sintered and also firmly bonded with said first type layer.

8. In a process as described in claim 1, the step of shaping said layers united by final sintering while still hot at temperatures exemplified by about 450° to below 900° C.

9. A process of manufacturing a layered armor composed of a number, two as a minimum, of layers or strata of different type material, a first type being ferrous, tough and hard and including in its manufacture a casting step, while the second type of material consists of a sintered hard metal composition obtained by sintering an initial mixture of hard particles selected from carbides, nitrides and borides of at least one element selected from the group consisting of tungsten, molybdenum, chromium, tantalum, niobium, vanadium, titanium, zirconium and boron, and a powdery cementing metal of lower melting point than said particles, said cementing metal always including an appreciable amount of iron group metal, comprising the steps of placing said completed first type layer in a die, depositing thereon a layer of said initial mixture, compacting said deposited layer upon said first type layer, and finally heating said layers to temperatures between about 900° to about 1350° C. until said second type layer is finally sintered and firmly bonded with said first type layer.

10. In a process as described in claim 9, the step of placing previous to final sintering a completed first type layer upon said second type layer deposited on the completed first type layer previously placed in the die.

11. In a process as described in claim 9, placing a completed first type layer of other than straight shape into a die, and depositing thereon at least one layer of said initial mixture admixed with

about 1% to 6% of a binder exemplified by organic and volatile binders.

12. A process of manufacturing a layered armor composed of a number, two as a minimum, of layers or strata of different type material, a first type being ferrous, tough and hard and including in its manufacture a casting step, while the second type of material consists of a sintered hard metal composition obtained by sintering an initial mixture of hard particles selected from carbides, nitrides and borides of at least one element selected from the group consisting of tungsten, molybdenum, chromium, tantalum, niobium, vanadium, titanium, zirconium and boron, and a powdery cementing metal of lower melting point than said particles, said cementing metal always including an appreciable amount of iron group metal, comprising the steps of continuously feeding a completed first type layer under means for depositing thereon a layer of an initial mixture for said second type layer and depositing said second type layer on said completed first type layer, feeding said layers into means for compacting said deposited layer upon said first type layer, thereafter successively passing said layers through heating zones of different degrees of temperature, in the first of which said deposited second type layer is heated to a temperature below about 700° to 900° C. and in the last of which said deposited layer is heated to final sintering temperature and thereby finally sintered and also firmly bonded with said first type layer.

13. A process of manufacturing a layered armor composed of a number, two as a minimum, of layers or strata of different type material, a first type being ferrous, tough and hard and including in its manufacture a casting step, while the second type of material consists of a sintered hard metal composition obtained by sintering an initial mixture of hard particles selected from carbides, nitrides and borides of at least one element selected from the group consisting of tungsten, molybdenum, chromium, tantalum, niobium, vanadium, titanium, zirconium and boron, and a powdery cementing metal of lower melting point than said particles, said cementing metal always including an appreciable amount of iron group metal, comprising the steps of continuously feeding a completed first type layer under means for depositing thereon a layer of an initial mixture for said second type layer and depositing said second type layer on said completed first type layer, passing said layers through means for compacting said deposited layer upon said first type layer, passing thereafter said layers through a heating zone wherein said deposited second type layer is heated to a temperature below about 700° to 900° C., passing thereafter said layers again through means for pressing them together, and finally passing said layers through a heating zone in which said deposited second type layer is finally sintered and also firmly bonded with said first type layer.

14. A process of manufacturing a layered armor composed of a number, two as a minimum, of layers or strata of different type material, a first type being ferrous, tough and hard and including in its manufacture a casting step, while the second type of material consists of a sintered hard metal composition obtained by sintering an initial mixture of hard particles selected from carbides, nitrides and borides of at least one element selected from the group consisting of tungsten, molybdenum, chromium, tantalum, niobium,

um, vanadium, titanium, zirconium and boron, and a powdery cementing metal of lower melting point than said particles, said cementing metal always including an appreciable amount of iron group metal, comprising the steps of continuously feeding a completed first type layer under means for depositing thereon a layer of an initial mixture for said second type layer and depositing said second type layer on said completed first type layer, feeding said layers into means for compacting said deposited layer upon said first type layer, feeding thereafter said layers into a heating device for finally sintering said second type layer upon said first type layer, and subjecting thereafter the continuously fed forward and united layers to a heat treatment according to a predetermined temperature-time curve in order to impart desired properties at least to said first type layer.

15. A process of manufacturing a layered armor composed of a number, two as a minimum, of layers or strata of different type material, a first type being ferrous, tough and hard and including in its manufacture a casting step, while the second type of material consists of a sintered

hard metal composition obtained by sintering an initial mixture of hard particles selected from carbides, nitrides, and borides of at least one element selected from the group consisting of tungsten, molybdenum, chromium, tantalum, niobium, vanadium, titanium, zirconium and boron, and a powdery cementing metal of lower melting point than said particles, said cementing metal always including an appreciable amount of iron group metal, comprising the steps of continuously feeding a completed first type layer under means for depositing thereon a layer of an initial mixture for said second type layer and depositing said second type layer on said completed first type layer, feeding said layers into means for compacting said deposited layer upon said first type layer, feeding subsequently said layers into a heating device for finally sintering said second type layer upon said first type layer, and subjecting thereafter the continuously fed forward, united and still hot layers to further shaping at temperatures between about 450° C. to below 900° C.

PAUL SCHWARZKOPF.